

## UNITED STATES PATENT OFFICE

2,297,698

## TREATING BIBULOUS PAPER

Richard D. Freeman, Midland, Mich., assignor to  
The Dow Chemical Company, Midland, Mich.,  
a corporation of Michigan

No Drawing. Application July 28, 1940,  
Serial No. 346,653

7 Claims. (Cl. 117—163)

This invention relates to the art of processing paper. It more particularly concerns an improved method of treating bibulous paper to increase the wet strength without materially decreasing the absorptivity thereof.

One of the chief disadvantages attendant use of the usual varieties of bibulous paper, such as toweling of the waterleaf variety, for example, is its tendency to disintegrate rapidly under the action of wiping wet hands. Various methods have been proposed for overcoming this serious disadvantage, but none have proven entirely satisfactory. For example, binding agents have been incorporated into the paper to increase its strength, but these so reduce the absorptive properties of the paper as to render it unsuitable for use as a toweling or for like purposes. In addition, the toweling of non-fibrous addition agents, such as regenerated cellulose, gelatine, urea-formaldehyde resins, glycerine, etc., while sometimes providing satisfactory strength or absorptive characteristics, has been found generally to yield a product which is either too stiff to be satisfactorily manipulated or one which becomes sticky or slippery when wet and thus unpleasant to the touch.

It is, therefore, the principal object of the present invention to provide a method of treating bibulous paper whereby the wet strength thereof may be substantially increased without materially decreasing its absorptive properties. Another object is to provide an easily manipulated paper toweling which is not too stiff and which does not become either sticky or slippery when wet. Other objects and advantages will be apparent as the description of the invention proceeds.

The foregoing objects may be accomplished and new and improved results obtained by coating commercial bibulous paper, such as that used in making paper toweling, for example, with a water solution of a mixture containing a minor proportion of a water-soluble cellulose ether and a major proportion of a mixture or compound of urea-formaldehyde and a polyhydric alcohol. Paper coated in this manner, after being dried and heated to set the resin, has markedly increased wet strength over those known in the art, and yet retains satisfactory absorptivity.

According to one embodiment of the invention, there is first prepared an approximately 5 per cent by weight solution in water of a mixture comprising between about 5 and 40 parts by weight of a water-soluble cellulose ether, from 50 to 95 parts of an urea-formaldehyde condensa-

tion product, and from 50 to 100 parts of a polyhydric alcohol. This solution may then be applied to toweling in any of the ways commonly known in the art, such as by spraying, brushing, dipping, or the like. The paper thus coated is then dried in air and heated to a temperature above 100° C. to set up the urea-formaldehyde resin. A catalyst, such as a trace of phosphoric acid, may be added to the composition to facilitate the setting up of the resin. After drying, the paper may be rolled or folded as desired, and is then ready for use. While the above proportions of ingredients give a generally satisfactory coating, maximum strength and absorptive properties are secured when the coating materials are in the ratio of approximately 5 to 15 parts of a water-soluble cellulose ether, 85 to 95 parts of urea-formaldehyde condensation product and 70 to 100 parts of polyhydric alcohol. This solution, when applied as a coating on bibulous paper, results in the formation of a product of exceptionally high wet strength and good absorptivity. In addition, paper coated with a solution of the type described is not unpleasant to the touch, i. e., is neither harsh nor slimy, even when wet.

Among suitable water-soluble cellulose ethers which may be used according to the invention are various alkyl celluloses, such as dimethyl cellulose; hydroxy alkyl celluloses, such as hydroxyethyl cellulose; alkali metal salts of carboxy-alkyl celluloses, such as sodium cellulose glycollate; etc.

The urea-formaldehyde condensation product and the polyhydric alcohol may be added to the composition as a mixture, or alternatively, a polyhydric alcohol-modified urea-formaldehyde resin may be used. Thus, I may use either a mixture of a simple urea-formaldehyde condensation product such as dimethylol urea with a polyhydric alcohol such as ethylene glycol or glycerol, or a resin containing ethylene glycol in chemical combination with urea and formaldehyde. Resins of this latter type are disclosed in U. S. Patent No. 2,168,477, to the assignee of Hodgins and Hovey.

In the appended claims, the expression "polyhydric alcohol-modified urea-formaldehyde resin" is intended to be generic to mixtures of a polyhydric alcohol and an urea-formaldehyde resin, as well as to those urea-formaldehyde resins which have been chemically modified with polyhydric alcohols during their manufacture.

The following examples illustrate the principle of the invention, but are not to be construed as limiting its scope.

## Example 1

Test strips 15 millimeters by 180 millimeters were cut from sheets of an ordinary roll of commercial paper toweling manufactured under the trade name "Wipemdry" and water solutions containing varying proportions of methyl cellulose and a glycol-modified urea-formaldehyde resin were then deposited upon the sample strips at various wet coating thicknesses in the range between 0.002 and 0.020 inch. All solutions used were of 5 per cent by weight concentration. The strips were then air dried, heated briefly to 105° C. to set the resin, and conditioned for 24 hours at 50 per cent relative humidity and 70° C. prior to testing. The water absorptivity of the strips was determined by the standard method of the Technical Association of Pulp and Paper Industry (T432M-36), as follows. The paper was placed on a 4-mesh screen and 0.01 milliliter of water at 20° C. was administered to the sheet from a graduated pipette. The required time in seconds was noted for the drop to be completely absorbed. The end point was taken as the point at which no light reflection was obtained from the water spot. The wet strength was determined by means of a Scott tensile strength tester, test strips being placed between the jaws of the machine and tension being applied to the strip until breakage occurred. Results obtained indicated that a solution containing approximately 10 parts by weight of methyl cellulose for each 90 parts by weight of a modified urea-formaldehyde resin imparted the most desirable properties to the toweling. Test strips coated with this solution had a relatively high degree of absorptivity and satisfactory strength characteristics. In addition, the surfaces of these strips were not slimy or unpleasant to the touch. However, sample strips of toweling coated with methyl cellulose alone had a slimy surface and a relatively low tensile strength. When a solution of glycol-modified urea-formaldehyde resin alone was applied to the test strips, considerable difficulty in casting was encountered due to the water-like viscosity of the solution. No improvement was noted in the paper strength. Results of the tests also indicated that a low viscosity cellulose ether imparts greater absorptivity to the treated paper than does a high viscosity cellulose ether when both are employed in the composite coating solutions herein claimed.

## Example 2

Tests were carried out on test strips prepared in a manner similar to those of Example 1 with solutions containing varying proportions of methyl cellulose and unmodified urea-formaldehyde resin. It was found that a test strip coated with a solution containing approximately 10 parts by weight of methyl cellulose for each 90 parts by weight of urea-formaldehyde had a satisfactory wet strength but unsatisfactory absorptivity. Increasing the methyl cellulose content of the solution did not improve the absorptivity of the test strips and tended to reduce their wet strength. However, in contrast, when 80 parts by weight of glycol was added to a solution containing 10 parts by weight of methyl cellulose and 90 parts by weight of urea-formaldehyde, a coated paper having satisfactory absorptivity and relatively high tensile strength was obtained.

As an indication of the degree of strength improvement accomplished by means of the herein

claimed method, the following representative comparative data are given:

|    |                                                                            | Wet strength pounds per inch width (average of several) | Absorptivity, seconds (average of several) |
|----|----------------------------------------------------------------------------|---------------------------------------------------------|--------------------------------------------|
| 10 | Bibulous paper (blank).....                                                | 0.6-1.1                                                 | 500-600                                    |
|    | Bibulous paper+methyl cellulose.....                                       | 0.35-0.52                                               | 140-200                                    |
|    | Bibulous paper+urea-formaldehyde resins.....                               | 1.5-2                                                   | 120-200                                    |
|    | Bibulous paper+methyl cellulose+urea-formaldehyde (unmodified).....        | 2-4                                                     | 600-900                                    |
| 15 | Bibulous paper+methyl cellulose+urea-formaldehyde (unmodified)+glycol..... | 1.7-2.7                                                 | 180-260                                    |
|    | Bibulous paper+methyl cellulose+glycol-modified urea-formaldehyde.....     | 2.2-2.8                                                 | 70-100                                     |

In the foregoing, the proportions of components in the treating solutions employed were those herein recited.

While the invention has been described with particular reference to treating paper toweling, it may also be applied to improve the wet strength without decreasing the absorptivity of other forms of bibulous paper, such as cleansing and toilet tissues, paper napkins, and the like.

Other modes of applying the principle of my invention may be employed instead of those explained, change being made as regards the method herein disclosed or the materials employed, provided the step or steps stated by any of the following claims be employed or the product claimed in any of the following claims be obtained.

I therefore particularly point out and distinctly claim as my invention:

1. A method of preparing absorptive paper products of high wet strength which comprises treating a bibulous paper base with a water solution whereof the solute comprises a minor proportion of a water soluble cellulose ether and a major proportion of a polyhydric alcohol-modified urea-formaldehyde resin, drying the so-coated paper, and heating the paper to a temperature of approximately 90° to 120° C. to set the resin.

2. A method of preparing absorptive paper products of high wet strength which comprises treating a bibulous paper base with a water solution whereof the solute comprises from 5 to 40 parts of a water soluble cellulose ether, from 50 to 95 parts of an urea-formaldehyde resin modified with from 50 to 100 parts of a polyhydric alcohol, drying the so-called paper and heating the paper to a temperature of approximately 90° to 120° C. to set the polyhydric alcohol-modified resin.

3. A method of preparing absorptive paper products of high wet strength which comprises treating a bibulous paper base with a water solution whereof the solute comprises from 5 to 15 parts of a water soluble cellulose ether, from 85 to 95 parts of an urea-formaldehyde resin modified with from 70 to 100 parts of a polyhydric alcohol, drying the so-coated paper and heating the paper to a temperature of approximately 90° to 120° C. to set the polyhydric alcohol-modified resin.

4. A method of preparing absorptive paper products of high wet strength which comprises treating a bibulous paper base with a water solution whereof the solute comprises from 5 to 40 parts of water soluble methyl cellulose, 50 to 95 parts of an urea-formaldehyde condensation product modified with from 50 to 100 parts of a polyhydric alcohol, drying the so-coated paper and heating the paper to a temperature of ap-

proximately 90° to 120° C. to set the polyhydric alcohol-modified resin.

5. A method of preparing absorptive paper products of high wet strength which comprises treating a bibulous paper base with a water solution whereof the solute comprises from 5 to 15 parts of water soluble methyl cellulose, from 85 to 95 parts of an urea-formaldehyde resin modified with from 70 to 100 parts of ethylene glycol, drying the so-coated paper and heating the paper 10 to a temperature of approximately 90° to 120° C. to set the polyhydric alcohol-modified resin.

6. Bibulous paper of improved wet strength bearing at least a superficial coating comprising a minor proportion of a water soluble cellulose ether and a major proportion of a polyhydric alcohol-modified urea-formaldehyde resin.

7. Bibulous paper of improved wet strength bearing at least a superficial coating comprising a minor proportion of water soluble methyl cellulose and a major proportion of glycol-modified urea-formaldehyde resin.

RICHARD D. FREEMAN.